

## UNITED STATES PATENT OFFICE

2,038,403

THERMO-ADHESIVE TEXTILE FABRIC  
AND PROCESS

Peter J. Ariende, Saylesville, R. I., assignor to  
Sayles Finishing Plants, Inc., Saylesville, R. I.,  
a corporation of Rhode Island

No Drawing. Application November 18, 1935,  
Serial No. 50,476

12 Claims. (Cl. 91—68)

The present invention relates to a thermo-adhesive textile fabric adapted for use as a lining.

An object of the invention is to produce a thermo-plastic and adhesive textile fabric which will adhere with great permanence to ordinary textile fabrics upon the application of heat and pressures characteristic of normal ironing.

The fabric of this invention combines for the first time in the art, so far as I am aware, the following characteristics, which are desirable in a lining for collars, cuffs, shirt bosoms and light weight, light colored textile fabrics in general:—

1. The fabric is entirely non-adhesive at room temperatures or thereabouts.
2. It becomes adhesive to ordinary textile fabrics at a temperature safely below the scorching point of the fabrics without the use of a solvent.
3. The adhesive bond produced does not break during repeated normal launderings.
4. If the adhesive bond is ruptured it can be restored by normal ironing.

5. The fabric remains colorless during all operations of manufacture and use.

6. The thermo-adhesive material does not penetrate through to the exterior surface of fabrics to which it is bonded.

This application is a continuation in part of my co-pending application, Ser. No. 756,311, filed December 6, 1934.

30 In making my fabric, I prepare a thermo-adhesive material by dissolving in one or more organic solvents, a solid alkyl-ortho-benzoyl-benzoate having not more than two carbon atoms in the alkyl radical (namely, methyl- or ethyl-ortho-benzoyl-benzoate) and a suitable cellulose derivative which is insoluble in water but soluble in the solvent or solvents for the alkyl-ortho-benzoyl-benzoate.

40 The following may be given as examples of such an adhesive:—

## Example #1

|                              | Per cent |
|------------------------------|----------|
| Cellulose acetate            | 13.6     |
| Acetone                      | 33.2     |
| Ethyl acetate                | 33.2     |
| Ethyl-ortho-benzoyl-benzoate | 20.0     |

## Example #2

|                               | Per cent |
|-------------------------------|----------|
| Cellulose acetate             | 13.5     |
| Acetone                       | 33.0     |
| Ethyl acetate                 | 33.0     |
| Methyl-ortho-benzoyl-benzoate | 20.5     |

## Example #3

|                              | Per cent |
|------------------------------|----------|
| Cellulose nitrate            | 13.5     |
| Acetone                      | 16.5     |
| Toluene                      | 16.5     |
| Ethyl acetate                | 33.0     |
| Ethyl-ortho-benzoyl-benzoate | 20.5     |

## Example #4

|                              | Per cent |
|------------------------------|----------|
| Ethyl cellulose              | 13.7     |
| Acetone                      | 33.7     |
| Ethyl acetate                | 33.6     |
| Ethyl-ortho-benzoyl-benzoate | 14.0     |
| Pigment                      | 5.0      |

While excellent results may be obtained with these specific compositions, it is to be understood that the percentages given may be varied and that other constituents may be substituted so long as they fall within the groups herein set forth.

Both methyl- and ethyl-ortho-benzoyl-benzoate may be used in the same composition, and more than one cellulose derivative of the class set forth may be used if desired.

Several coats of my thermo-adhesive mixture may be applied, for example by means of a coating machine, to either one or both sides of a textile fabric. The coated fabric is then dried, preferably at a temperature of about 110° F. This removes the solvent and leaves the fabric coated with a thermo-adhesive composition. In the case of the composition of Example 1 above, for instance, the dried coating on the fabric would comprise approximately 40% cellulose acetate and approximately 60% ethyl-ortho-benzoyl-benzoate.

The dried fabric has all the above-enumerated desirable characteristics.

This coated fabric will adhere tenaciously to other fabrics when they are placed together and ironed with a heated iron at temperatures well below the scorching point of the fabrics.

A very advantageous result may be obtained by pretreating the fabric, before it is coated with the thermo-adhesive material, with a dressing or sizing of a material, preferably insoluble in water, such as casein, regenerated cellulose, or the like, and if desired, with a filler also, such as talc, clay or the like.

For example, a suitable fabric, after having been boiled and bleached in the usual manner, may be treated (for example by immersion) with a viscose solution containing 4% cellulose. The cellulose may be regenerated with a sulphuric acid

bath and the fabric washed free from acid and dried. The fabric may then be coated with my thermo-adhesive composition.

While my novel thermo-adhesive textile fabric is adapted to general use for the production of duplex or multi-ply fabrics, it is particularly useful as a lining in the production of composite fabrics to be made into collars, cuffs, shirt bosoms, etc., which it is desired shall be especially resistant to wilting, massing and wrinkling. During normal launderings the adhesion between the lining and adjacent textile fabric remains intact. The lining makes such laundered article sufficiently stiff so that the use of starch is not necessary.

A particular advantage of my fabric when used as a lining is that the bond between the lining and the adjacent fabric not only withstands repeated normal launderings, but if because of abnormal conditions the bond becomes loose or broken, all that is necessary to restore the bond and re-adhere the lining to the fabric is to iron again in the usual way. This property of the lining clearly distinguishes it from those linings which are made with preparations containing synthetic resins. The adhesive bonds of such latter linings I have found to be objectionable. Either they are incapable of withstanding repeated normal launderings without breaking or, if the bonds are capable of withstanding such launderings, they cannot be restored by merely ironing again if the bonds are once broken by abnormal conditions.

Another advantage of my fabric when used as a lining is that to render it properly adhesive only ordinary ironing is required and no treatment with organic solvent is necessary. The use of such a solvent is objectionable in the manufacture of collars, cuffs, shirts, etc.

I claim:

40. 1. A thermo-adhesive textile fabric lining comprising a fabric coated with a composition comprising an alkyl-ortho-benzoyl-benzoate having not more than two carbon atoms in the alkyl radical, and a cellulose derivative which is insoluble in water but soluble in a solvent for the alkyl-ortho-benzoyl-benzoate, said lining having the properties of adhering tenaciously to other textile fabrics after heating under pressure at a temperature below the scorching point of the fabrics, of providing an adhesive bond between itself and such other fabrics, which bond is capable of withstanding repeated launderings and if ruptured is capable of restoration by the application of heat and pressure, and of withstanding discoloration during normal manufacture and use.

2. As a new article of manufacture, a thermo-adhesive textile fabric lining comprising a fabric coated with a thermo-adhesive composition comprising an ester of the alkyl-ortho-benzoyl-benzoate class having not more than two carbon atoms in the alkyl radical and a cellulose derivative which is insoluble in water and soluble in a solvent for the said alkyl-ortho-benzoyl-benzoate.

65. 3. A thermo-adhesive textile fabric comprising a fabric coated with a composition comprising an alkyl-ortho-benzoyl-benzoate selected from the group consisting of methyl-ortho-benzoyl-benzoate and ethyl-ortho-benzoyl-benzoate, and a cel-

lulose derivative which is insoluble in water but soluble in a solvent for the alkyl-ortho-benzoyl-benzoate.

4. A process of preparing a fabric lining for a textile material composed of two or more sheets, which process comprises dissolving cellulose acetate and an alkyl-ortho-benzoyl-benzoate having not more than two carbon atoms in the alkyl radical in one or more volatile organic solvents, coating said fabric with said solution and drying the coated fabric to remove the solvent, whereby thermo-adhesive properties are imparted to the fabric.

5. A thermo-adhesive textile fabric adapted for use as a lining comprising a fabric coated with a composition comprising cellulose acetate and ethyl-ortho-benzoyl-benzoate, said fabric having the properties of adhering tenaciously to other textile fabrics after heating under pressure at a temperature below the scorching point of the fabrics, of providing an adhesive bond between itself and such other fabrics, which bond is capable of withstanding repeated launderings and if ruptured is capable of restoration by the application of heat and pressure, and of withstanding discoloration during normal manufacture and use.

6. A thermo-adhesive textile fabric comprising a fabric coated with a thermo-adhesive composition comprising cellulose acetate and ethyl-ortho-benzoyl-benzoate.

7. A thermo-adhesive textile fabric lining comprising a fabric coated with a thermo-plastic composition comprising approximately 40% of cellulose acetate and approximately 60% of ethyl-ortho-benzoyl-benzoate.

8. A thermo-adhesive textile fabric comprising a fabric coated with a composition comprising methyl-ortho-benzoyl-benzoate and a cellulose derivative which is insoluble in water but soluble in a solvent for said methyl-ortho-benzoyl-benzoate.

9. A thermo-adhesive textile fabric comprising a fabric coated with a thermo-adhesive composition comprising cellulose acetate and methyl-ortho-benzoyl-benzoate.

10. A lining consisting of a textile fabric filled with a water-insoluble sizing, with or without a mineral filler, and coated with a thermo-adhesive material comprising an alkyl-ortho-benzoyl-benzoate having not more than two carbon atoms in the alkyl radical, and a cellulose derivative insoluble in water but soluble in a solvent for said alkyl-ortho-benzoyl-benzoate.

11. A lining material consisting of a textile fabric sized with regenerated cellulose and coated with a thermo-adhesive material comprising an alkyl-ortho-benzoyl-benzoate selected from the group consisting of methyl-ortho-benzoyl-benzoate and ethyl-ortho-benzoyl-benzoate, and a cellulose derivative which is insoluble in water but soluble in a solvent for said alkyl-ortho-benzoyl-benzoate.

12. A lining consisting of a textile fabric filled with a water-insoluble sizing, with or without a mineral filler, and coated with a thermo-adhesive material comprising cellulose acetate and ethyl-ortho-benzoyl-benzoate.

PETER J. ARIENTE.